



US005985046A

# United States Patent [19]

Serafin et al.

[11] Patent Number: **5,985,046**[45] Date of Patent: **\*Nov. 16, 1999**

[54] **PROCESS FOR MAKING CLEAR COATED ALUMINUM ALLOY LIGHTING SHEET**

[75] Inventors: **Daniel L. Serafin**, Wexford, Pa.; **Paula A. Hinds**, Lawrenceville, Ga.; **Paul B. Schultz**, Export, Pa.; **Albert L. Askin**, Lower Burrell, Pa.; **Robert E. Bombalski**, Brackenridge, Pa.

[73] Assignee: **Aluminum Company of American**, Pittsburgh, Pa.

[\*] Notice: This patent is subject to a terminal disclaimer.

[21] Appl. No.: **09/037,696**

[22] Filed: **Mar. 10, 1998**

## Related U.S. Application Data

[63] Continuation-in-part of application No. 08/625,583, Mar. 28, 1996, Pat. No. 5,725,683.

[51] **Int. Cl.<sup>6</sup>** ..... **C23C 22/00**

[52] **U.S. Cl.** ..... **148/243; 148/256; 148/265; 148/275; 427/385.5; 427/387**

[58] **Field of Search** ..... 148/243, 275, 148/265, 256; 427/385.5, 387, 407.1, 409, 419.1, 428

[56]

## References Cited

### U.S. PATENT DOCUMENTS

4,490,184 12/1984 Forcht et al. ..... 148/275  
5,478,414 12/1995 Mozelewski et al. ..... 148/265

*Primary Examiner*—Prince Willis

*Assistant Examiner*—Andrew L. Oltmans

*Attorney, Agent, or Firm*—Glenn E. Klepac

[57]

## ABSTRACT

A process for making an aluminum alloy lighting sheet product having a reflective surface protected by a UV-stable polymer coating. An aluminum alloy sheet is chemically brightened in an aqueous acidic solution, conversion coated, and then coated with a UV-stable polymer. Alternatively, an aluminum alloy sheet is chemically etched in an aqueous alkaline solution, conversion coated, and then coated with a UV-stable polymer. The UV-stable polymer may be clear or it may contain about 0.5–10 wt. % amorphous silica particles and polytetrafluoroethylene particles. In another embodiment, an aluminum alloy sheet surface is cleaned, chemically conversion coated and then coated with a coating composition containing a UV-stable polymer and 0.5–10 wt. % silica particles and polytetrafluoroethylene particles, both having an average size of about 0.5–5 microns.

**15 Claims, No Drawings**

# PROCESS FOR MAKING CLEAR COATED ALUMINUM ALLOY LIGHTING SHEET

## RELATED APPLICATION

This application is a continuation-in-part of U.S. Ser. No. 08/625,583, filed Mar. 28, 1996, now U.S. Pat. No. 5,725,683, issued Mar. 10, 1998.

## FIELD OF THE INVENTION

The present invention relates to methods and compositions for making corrosion resistant aluminum alloy sheet products having a specular or diffuse appearance and a highly reflective surface, without anodizing the surface.

## BACKGROUND OF THE INVENTION

Although aluminum is ordinarily considered a bright metal, the surface appearance is generally specified by the customer as either having a semi-specular (matte-like) finish or a specular finish. In lighting applications, it is especially desirable that the aluminum have a highly reflective surface, regardless of the specularity of the finish. As used herein, the term "total reflectance" refers to the amount of incident light striking a surface that is reflected in any direction, and the term "highly reflective" refers to a surface which reflects 80% or more. As used herein, the term "specular reflectance" refers to reflectance measured at an angle which is equal to the angle of incidence. The matte-like or semi-specular finish is defined as an appearance which has a specular reflectance of less than 40%, while the specular finish refers to the finish which has a specular reflectance of greater than 40%, both measured at 30 degrees from normal incident light, per ASTM E-430.

Some known processes for polishing aluminum to produce a highly reflective surface include chemical polishing or electropolishing, both generally carried out in an acidic bath. After polishing, the surface must be treated again to render it resistant to corrosion. In the prior art, corrosion resistance has generally been imparted to aluminum alloy surfaces by anodizing and then coating with a polymer layer. Nikaido et al U.S. Pat. No. 3,945,899 is an example of one prior art reference disclosing anodization of an aluminum alloy surface followed by coating, preferably with an organic polymer such as an acrylic resin or acrylic modified polyester.

Anodizing processes have been practiced commercially on aluminum lighting sheet products for several years. Although anodized surfaces are chemically stable and resistant to corrosion, the processes are expensive. In addition, anodized aluminum alloy surfaces are often subject to some iridescence and to some oxide crazing during subsequent forming or exposure to elevated temperatures.

A principal objective of the present invention is to produce an aluminum sheet having a highly reflective and corrosion-resistant surface, in either a specular or semi-specular finish, without anodizing the surface. The term "corrosion resistant" refers to a product that does not delaminate, peel or significantly yellow or whiten when exposed to 1,000 hours of cycled condensing humidity and UV light, per ASTM G-53.

A related objective of the invention is to provide a process for making aluminum alloy sheet with improved characteristics, such as improved resistance to crazing and improved control of iridescence while maintaining acceptable levels of scratch and dust resistance, formability, appearance, optical performance and long term durability, compared with prior art processes relying upon anodizing.

Additional objectives and advantages of our invention will become apparent to persons skilled in the art from the following detailed description.

## SUMMARY OF THE INVENTION

In accordance with the present invention, there is provided a process for making an aluminum alloy sheet product having a reflective surface protected by a conversion coating and a polymer coating.

10 Aluminum sheet material of the invention is preferably made from an aluminum alloy. As used herein, the term "aluminum alloy" refers to an alloy containing about 90% or more aluminum, and one or more alloying elements. When alloying is necessary for mechanical performance, the preferred alloying elements are magnesium, usually comprising about 0.5 to 10 wt. % of the alloy, and manganese, usually provided at about 0.15 to 2 wt. % of the total alloy. Various aluminum alloys in sheet form are suitable for the practice of the present invention, including the alloys of the 1000, 20 3000 and 5000 series (Aluminum Association designations). Appropriate tempers include H1x, H2x, H3x and O-tempers (Aluminum Association designations). Aluminum-magnesium alloys of the AA5000 series are preferred, especially the AA5000 series alloys containing about 1.5 wt. % or less magnesium.

25 A suitable aluminum alloy would be a bright-rolled alloy which has a surface roughness of 0 to 3 micro-inches, a preferred mill finish which has a surface roughness of 4 to 13 micro-inches and a mill finish with a surface roughness of 14 or greater micro-inches. Alternatively, the sheet may be rolled with a textured roll to produce a surface roughness ( $R_a$ ) of about 10-25 micro-inches.

30 Some suitable compositions include the 1050, 1100, 1085, 3003, 3004, 3005, 5005, 5050, 5052, 5252 and 5657 aluminum alloys (Aluminum Association series).

35 A particularly preferred AA 5005 alloy contains about 0.5-1.1 wt. % Mg, 0.07-0.30 wt. % Si, 0.10-0.7 wt. % Fe, 0.03-0.20 wt. % Cu, 0.20 wt. % max. Mn, 0.10 wt. % max. Cr, 0.25 wt. % max. Zn, 0.15 wt. % max. other alloying elements and impurities, and remainder Al. More preferably, the alloy contains about 0.65-0.80 wt. % Mg, 0.07-0.09 wt. % Si, 0.10-0.17 wt. % Fe, 0.03-0.06 wt. % Cu, 0.010 wt. % max. Mn, 0.05 wt. % max. Cr, 0.10 wt. % max. Zn, 0.10 wt. % max. other alloying elements and impurities, and remainder Al.

40 For the specular product, the bright-rolled sheet may be immersed in an acidic cleaning/brightening bath to remove the lubricant film and to further improve the surface quality. 45 The cleaning/brightening bath is preferably an aqueous solution containing phosphoric acid, sulfuric acid, nitric acid, dissolved aluminum and a copper salt that is maintained at a temperature above 150° F. A preferred bath temperature is about 200° F. Likewise, a suitable aqueous solution is known to contain phosphoric acid, nitric acid, dissolved aluminum and a copper salt.

50 The cleaned and brightened sheet may be desmutted, preferably in an aqueous acidic solution containing nitric or sulfuric acid or a mixture of sulfuric acid and chromic acid. 55 The nitric or sulfuric desmutting solutions are generally used at ambient temperature, and the sulfuric-chromic acid solution is preferably heated to about 160° to 180° F.

60 For the matte-like, semi-specular product, the bright-rolled, preferred mill finish or mill-finish sheet is etched in an alkaline bath. A preferred caustic etching solution contains 50 g/L sodium hydroxide and an organic wetting agent, maintained at a temperature of about 150° to 160° F.

Commercially available alkaline etching solutions containing sodium hydroxide or potassium hydroxide or mixtures thereof are also suitable. One alternative treatment includes cleaning and etching the sheet in a solution containing phosphoric acid. After etching, the sheet may be desmutted, preferably in a solution containing citric acid and nitric acid. Alternatively, the sheet may be desmutted in a 20 wt. % sulfuric acid solution.

For both the specular and semi-specular finishes, a conversion coating is next applied to the sheet in order to assure good adhesion of the polymer coating and improved corrosion resistance of the final product. Both chrome-containing and chrome-free conversion systems are suitable. The chrome conversion coating generally contains a chromate and a phosphate. Some known non-chromate conversion coatings are solutions containing zirconate, titanate, molybdate, tungstate, vanadate and silicate ions, generally in combination with hydrogen fluoride or other fluoride compounds.

The conversion coated sheet may be rinsed and then dried thoroughly before it is spray coated or roll coated with a solution of a curable polymer. Some suitable polymers include polyesters, such as polyethylene terephthalate (PET) and polybutylene terephthalate (PBT), polyurethanes, polyvinyl chloride, nylon, polyolefins and various acrylics which are stable upon long-term exposure to ultraviolet (UV) radiation. A UV-stable polyester is particularly preferred. When a highly reflective finish is desired, the UV-stable polymer is preferably a polyester or acrylic that does not substantially diminish surface brightness.

The polymer coating is preferably dissolved in organic solvents such as methyl isobutyl ketone (MIBK) or methyl ethyl ketone (MEK) or butyl cellosolve, for example, in a concentration of about 35 wt. %. The solution is preferably roll coated or sprayed onto the sheet to produce a coating thickness of about 0.1 to 2 mils, preferably about 0.1 to 1 mil. A polymer coating thickness of about 0.2 to 0.3 mils is usually sufficient for most indoor applications.

The polymer coating preferably contains particulate additives in order to simulate the appearance of commercially available, semi-specular sheet products. The coating usually contains about 0.5 to 10 wt. % of such additives. A particularly preferred coating contains a combination of silica particles and polytetrafluoroethylene particles, both in the 0.5 to 5 micron average size range. Surprisingly, silica particles alone were not capable of producing the desired appearance.

An alternative suitable process for producing a semi-specular finish is to clean the aluminum bright-rolled, preferred mill finish or mill-finish sheet, with or without a chemical etch or a chemical brightening, apply the conversion coating, and then to apply a polymer coating which contains silica and polytetrafluoroethylene particles in proportions of about 0.5 to 10 wt. %.

The polymer-coated sheet is heated in an oven to cure the polymer. The sheet will reach a peak cure temperature of about 400° to 500° F.

A particularly preferred 5005 alloy sheet is prepared from an ingot that is cast and homogenized according to conventional practice. The ingot is cast, scalped and then homogenized at an elevated temperature, typically at about 800° to 1050° F. for 2 to 24 hours.

In conventional practice, the homogenized ingot is next hot rolled and cold rolled to a sheet of desired thickness which is then partially annealed and slit to a predetermined width. We have found that a sheet having an improved

surface appearance is obtained by hot rolling, annealing, and then cold rolling instead of such conventional practice. Optionally, the sheet may be partially annealed after it is cold rolled.

As used herein, the term "hot rolling" refers to rolling that takes place at a metal entry temperature of about 450° to 1000° F. (232 to 538° C.) for aluminum alloys. Hot rolling is typically used to reduce slabs of aluminum alloy material several inches thick into sheets having a thickness of about 0.10 inch to 0.25 inch and typically about 0.125 inch (0.32 cm). After hot rolling, the metal exit temperature is in the range of about 300° to 600° F., preferably about 300° to 400° F.

The term "cold rolling" refers to rolling in which metal entry temperature ranges from ambient temperature to about 150° F. (54° C.) for aluminum alloys. Cold rolling is typically used to reduce sheets of aluminum alloy material to sheets having the desired thickness and surface finish.

The term "annealing" refers to heating in an oven at temperatures of about 600° to 900° F. for about 1 to 24 hours. The annealing temperature is preferably greater than the metal temperature at exit from the hot rolling process, and more preferably in the range of about 600° to 700° F.

The term "partial annealing" refers to heating in an oven at a temperature of about 300° to 500° F. for about 1 to 24 hours. Partial annealing may be employed to provide desired mechanical properties and formability in the sheet product.

In a particularly preferred embodiment, a slab of 5005 alloy having a thickness of about 20 inches (50 cm) is hot rolled to a thickness of less than 0.30 inch, preferably about 1/8 inch (0.32 cm). The metal is then annealed at 600° to 650° F. for 2 hours. The sheet is then cold rolled. Optionally, the sheet is annealed after the first cold rolling pass and then cold rolled again. Upon completion of cold rolling, the sheet may be partially annealed at 300° to 500° F. for about 6 hours. A particularly preferred partial annealing temperature is about 400° F.

The metal thickness, after cold rolling, ranges from 0.010 to 0.072 inch and is preferably about 0.016 to 0.025 inch.

The hot rolled sheet has a highly fragmented grain structure that ordinarily survives even after cold rolling. We have found that annealing the sheet after hot rolling and before cold rolling causes the grain structure to recrystallize into a shorter, less striated and more equiaxed grain structure. After the sheet is cold rolled to a lesser thickness, it remains free of the long grains responsible for streaky, directional appearance in the final polymer coated product. Appearance of the polymer-coated sheet is improved, both when the sheet is conversion coated and then polymer coated or when it is anodized.

#### DETAILED DESCRIPTION OF THE PREFERRED EMBODIMENTS

For the specular finish, the bright-rolled sheet may be immersed in an aqueous cleaning/brightening bath. One such bath may contain about 75 wt. % phosphoric acid, 15 wt. % sulfuric acid, 2 to 3 wt. % nitric acid and about 800-1000 ppm copper salts. The bath temperature is 200° F. One such other bath is an aqueous solution containing 80-85 vol. % phosphoric acid, 2 to 3 wt. % nitric acid, 10 to 40 ppm dissolved aluminum and 50 to 200 ppm copper salts. The cleaned and brightened sheet may then be desmutted in an aqueous solution containing about 50 wt. % nitric acid. Desmutting removes residual copper and oxides remaining on the sheet after cleaning and brightening.

For the semi-specular finish, a bright rolled, preferred mill finish or mill-finish sheet may be etched in an alkaline bath.

The preferred caustic etching solution contains 50 g/L sodium hydroxide and an organic wetting agent, maintained at a temperature of about 150° to 160° F. After etching, the sheet may be desmutted, preferably in 20 wt. % sulfuric acid solution.

The desmutted sheet is conversion coated, preferably in a solution containing chromate and phosphate ions. A commercially available BETZ 1904 conversion coating solution is particularly suitable. A BETZ 1903 conversion coating solution that is chromate free also performs well. The BETZ 1904 and BETZ 1903 conversion coating solutions are available from Betz Laboratories, Inc. of Trevose, Pa. The conversion coating solution, when not a dried-in-place coating, is rinsed, preferably in deionized water, and then dried thoroughly before polymer coating.

A particularly preferred UV-stable polyester is roll coated on the sheet from a 35 wt. % solution containing MIBK or MEK. The preferred coating thickness is about 0.2 to 0.3 mil.

The semi-specular finish may also be obtained by etching the bright-rolled, preferred mill finish, or mill-finish sheet in an aqueous alkaline bath, and subsequently conversion coating, then coating the sheet with a polymer coating which contains silica particles and polytetrafluoroethylene particles. The preferred caustic etching solution contains 50 g/L sodium hydroxide and an organic wetting agent, maintained at a temperature of about 150° to 160° F. After etching, the sheet may be desmutted, preferably in 20 wt. % sulfuric acid solution. The final polymer coating contains silica particles in concentrations of about 0.5 to 10 wt. %, preferably about 2 wt. %. The silica particles are preferably amorphous silica having an average particle size of about 0.5–5 microns. The preferred coating also contains about 0.5 to 1.0 wt. % polytetrafluoroethylene particles having an average size of about 1 micron.

The semi-specular finish may also be obtained by brightening the bright-rolled, preferred mill finish, or mill-finish sheet in an aqueous cleaning/brightening bath, and subsequently conversion coating, and then coating the sheet with a polymer coating which contains silica particles. One such bath may contain about 75 wt. % phosphoric acid, 15 wt. % sulfuric acid, 2 to 3 wt. % nitric acid and about 800 to 1000 ppm copper salts. The bath temperature is 200° F. Another such bath is an aqueous solution containing 80 to 85 vol. % phosphoric acid, 2 to 3 wt. % nitric acid, 10 to 40 ppm dissolved aluminum, and 50 to 200 ppm copper salts. The cleaned and brightened sheet may then be desmutted in an aqueous solution containing about 50 wt. % nitric acid. Desmutting removes residual copper and oxides remaining on the sheet after cleaning and brightening. The final polymer coating contains silica and polytetrafluoroethylene particles in a total concentration between about 0.5 and 10 wt. %. A particularly preferred polymer coating contains about 1.5 wt. % silica particles together with about 0.5 to 1.0 wt. % polytetrafluoroethylene particles. The silica particles are preferably amorphous silica with an average particle size of about 0.5 to 5 microns and the polytetrafluoroethylene particles have an average size of about 1 micron.

The semi-specular finish may also be obtained by conversion coating, and then coating the sheet with a polymer coating which contains silica particles and polytetrafluoroethylene particles in a total concentration between about 0.5 and 10 wt. %. A particularly preferred polymer coating contains about 1.5 wt. % silica particles together with about 0.5 to 1.0 wt. % polytetrafluoroethylene particles. The silica particles are preferably amorphous silica with an average

particle size of about 0.5 to 5 microns and the polytetrafluoroethylene particles have an average size of about 1 micron.

The polymer-coated sheet is heated in an oven to cure the polymer. A peak cure temperature of about 400° to 500° F. is used.

Persons skilled in the art will understand that numerous variations and changes can be made in the preferred embodiment of our invention described above without departing from the spirit and scope of the following claims.

What is claimed is:

1. A process for making an unanodized aluminum alloy sheet product having a reflective surface protected by a polymer coating, comprising:
  - (a) chemically brightening a surface of an unanodized aluminum alloy sheet by immersing said surface in an aqueous acidic solution containing a copper salt, achieving a total reflectance of greater than 89%;
  - (b) without anodizing said sheet, chemically conversion coating the brightened surface to generate an adherent film of a metal compound;
  - (c) coating the brightened surface with a polymer by contacting said surface with a solution comprising a UV-stable polymer dissolved in an organic solvent and then evaporating said solvent; and
  - (d) curing the polymer-coated surface at an elevated temperature.
2. The process of claim 1 further comprising:
  - (e) rinsing the conversion-coated surface after step (b) and drying to leave a dry brightened surface.
3. The process of claim 1 wherein the UV-stable polymer coated onto said surface in step (d) is a polyester or acrylic that does not substantially diminish surface brightness.
4. The process of claim 1 wherein said polymer contains silica particles having an average size of about 0.5–5 microns.
5. The process of claim 1 wherein the UV-stable polymer coated onto said surface in step (d) contains polytetrafluoroethylene particles having an average size of about 0.5–5 microns.
6. The process of claim 1 wherein the polymer-coated surface of step (e) has a coating thickness of about 0.1–1 mil.
7. The process of claim 1 wherein the aluminum alloy sheet comprises an alloy of the AA1000, 3000 or 5000 series.
8. A process for making an unanodized aluminum alloy sheet product having a reflective surface protected by a polymer coating, comprising:
  - (a) etching a surface of an unanodized aluminum alloy sheet by immersing said surface in a caustic etching solution, said sheet having total reflectance greater than 89% after said etching;
  - (b) chemically conversion coating the etched surface to generate an adherent film of a metal compound;
  - (c) coating the etched surface with a UV-stable polymer dissolved in an organic solvent containing polytetrafluoroethylene particles having an average size of about 0.5–5 microns; and
  - (d) curing said UV-stable polymer by heating.
9. The process of claim 8 wherein said UV-stable polymer is a polyester or acrylic that does not substantially diminish surface brightness.
10. The process of claim 8 wherein said organic solvent also contains silica particles having an average size of about 0.5–5 microns.
11. A process for making an unanodized aluminum alloy sheet product having a reflective surface protected by a polymer coating comprising:

- (a) cleaning a surface of an unanodized aluminum alloy sheet to remove a lubricant film residue, thereby to obtain a cleaned sheet surface having total reflectance greater than 89% after said cleaning;
- (b) chemically conversion coating the cleaned sheet surface to generate an adherent film of a metal compound;
- (c) coating the conversion coated sheet surface with a coating composition comprising a UV-stable polymer and silica particles and polytetrafluoroethylene particles each having an average size of about 0.5-5 microns.

- 12. The process of claim 11 wherein step (c) comprises roll coating said coating composition onto said sheet surface and said UV-stable polymer is dissolved in an organic solvent.
- 5 13. The process of claim 11 further comprising:
  - (d) curing said UV-stable polymer in the coating composition at an elevated temperature.
- 14. The process of claim 1 wherein said aqueous acidic solution contains about 50-1000 ppm of the copper salts.
- 10 15. The process of claim 8 wherein said caustic etching solution contains sodium hydroxide or potassium hydroxide or a mixture thereof.

\* \* \* \* \*